

## UNITED STATES PATENT OFFICE

2,089,948

## TEXTILE FABRIC

William Alexander Dickie and Robert Wighton  
 Moncrieff, Spondon, near Derby, England, as  
 signors to Celanese Corporation of America,  
 a corporation of Delaware

No Drawing. Application May 17, 1932, Serial  
 No. 611,924. In Great Britain June 4, 1931

14 Claims.

(Cl. 28—1)

This invention relates to the manufacture of textile fabrics and textile yarns suitable for incorporation therein and is more particularly concerned with the production of fabrics exhibiting crépe effects, especially from highly twisted cellulose ester or ether yarns.

Textile materials exhibiting crépe effects have long been obtained by employing in their construction highly twisted yarns of natural silk in the gummed state, the crépe effects appearing more particularly when the fabric is subjected to scouring in an aqueous bath. The fabrics obtained by this process have long been highly valued on account of their pleasing appearance and handle. The production of crépe fabrics in an analogous manner by the use of highly twisted yarns of cellulose acetate filaments has however been accompanied by very considerable difficulties. In many cases it is found that little or no crépe effect is obtained unless a very considerable degree of twist is imparted to the crépe threads. Further, when this degree of twist is sufficient to lead to the production of crépe effects comparable with those obtainable by means of natural silk, it is found that the strength of the resulting fabrics is frequently so low as to render them commercially valueless.

In U. S. application S. No. 523,930 filed 19th March, 1931, we have described an improved method of obtaining crépe fabrics with the aid of highly twisted cellulose acetate yarns. According to that specification the requisite high degree of twist is applied in two or more stages instead of in a single stage, as commonly practised. In this manner considerably improved results may be obtained, particularly as regards the strength of the finished fabrics in the direction of the highly twisted yarns.

We have now found that in utilizing highly twisted cellulose acetate yarns in the manufacture of crépe fabrics a further great improvement, particularly as regards the strength of the finished fabrics, may be effected by subjecting the yarn to the action of water vapour before at least part of the crépe twist is applied thereto. For example a cellulose acetate yarn of about 100 denier and containing about 25 filaments may be twisted to 25 to 30 turns per inch or more and then subjected to the action of steam at about 60—105° C., i. e. under a pressure below or slightly above that of the atmosphere. The so treated yarn is thereafter twisted to 60—70 turns per inch and utilized as the weft of a fabric, pairs of picks of right-hand twist alternating with pairs of picks of left-hand twist. The fabric may then be

scoured and finished, whereupon a fabric exhibiting excellent crépe effects and of very good properties as regards strength may be obtained. If the treatment with steam is omitted the resulting fabrics may exhibit a serious reduction in strength in the direction of the highly twisted 5 yarns.

In the manufacture of the crépe threads in accordance with our invention, the requisite high degree of twist is thus applied in at least two 10 stages with intermediate treatment of the yarn with water vapour. If desired the twisting may be accomplished in three or more stages, the yarn being treated with water vapour between 15 any or all of the stages. Further, if desired, the 15 yarn may be subjected, in addition, to water vapour treatment before twisting or after the total amount of twist has been applied.

The degree of twist employed in the crépe threads may vary within wide limits and according to the nature of the yarn and of the filaments contained therein. Thus, for instance, a total twist of from 55 to 65 or 70 turns per inch may be employed, though higher twist may be employed if desired, for example a twist of 80—85 25 or more turns per inch. Yarn composed of fine filaments is advantageous in that it admits of the use of a very high degree of twist. In this connection reference may be made to U. S. application S. No. 523,931, filed 19th March, 1931. 30

The total twist may be applied either in equal or in unequal stages. Thus, where twisting is to be effected in two stages, half the twist may be applied in each, or a small or large proportion in the first stage and in the second stage the corresponding proportion required to give the desired total twist. Thus, for instance, where the total twist is to be 65 turns per inch, the yarn may first be twisted to 10 turns per inch, then steamed, and thereupon an additional 55 turns 40 per inch applied to give the necessary total twist. Again, if desired 40 turns per inch may first be applied and 25 turns per inch in the second stage. In an analogous manner when three or more stages are employed the twist may be divided between the various stages in any desired manner. As indicated previously, however, in the case of 45 yarn of about 100 denier and containing about 25 filaments very good results may be obtained 50 by applying about 25 turns per inch in the first stage.

If desired any or all of the twist applied may be irregular in character as described in U. S. application S. No. 538,486, filed 19th May, 1931. 55

In practice, it has been found particularly advantageous to apply in the first place a degree of twist of the order of that necessary to cause a close packing of the filaments of the yarn and 5 then to treat the latter with water vapour and thereafter to impart the degree of twist necessary to give rise to crêpe effects of the desired character. In the case of 100 denier 26 filament yarn the desired close packing is secured by the application of about 25 turns per inch. It will be 10 appreciated that the exact degree of twist necessary to give the desired close packing of the filaments is dependent in any particular case on the total denier of the yarn and the number of the 15 filaments of which it is composed. Thus for yarns of a given total denier the twist required to effect close packing is greater the smaller the number of filaments. Again, for yarns containing a given number of filaments the desirable first stage twist 20 varies inversely as the diameter of the filaments or the square root of the filament denier. In general for yarns of between 70 and 170 denier and containing from 25 to 70 filaments the degree of twist applied before the wetting operation will be 25 between about 10 and 30 turns per inch.

The twisting of the yarns may be effected in any convenient manner. It has been found advantageous however, particularly when applying the second or subsequent stage of twist, to utilize 30 twisting devices of the type in which the yarn is twisted as it is drawn off from a rotating package and to prevent the applied twist running back to the bobbin. This result may very conveniently be attained by means of the device described in U. S. 35 Patent No. 1,784,581.

The crêpe effects obtained appear to be dependent chiefly upon the degree of twist imparted after the steam treatment and are to some extent independent of the degree of twist applied before 40 the steam treatment particularly if the said degree of twist is not much below that required to effect close packing of the filaments. It has in fact been found that the character or extent of the crêpe effects finally obtained in the fabrics may be controlled to some extent by varying the proportion of twist applied after a steaming treatment. The amount of twist imparted in the final stage or stages following packing of the filaments into a firm thread will thus depend to a certain 45 extent on the denier of the yarns and on the type of crêpe effect to be produced. In general a good figure is obtained on the fabrics by the use of a total twist of 60-65 to upwards of 85 turns per 50 inch.

In the treatment of the yarns in accordance with the present invention, the steam may be employed under any desired pressure and at any desired temperature, for example at pressures below or slightly above that of the atmosphere, and 55 at temperatures corresponding to the boiling point of water at those pressures. The steam may be dry, saturated, or wet. Very good results may be obtained for instance by using steam at pressures up to 5 lbs. per square inch below or above atmospheric pressure, though higher pressures, for example 10-20 lbs. per square inch or more, may be used if desired.

The operation of treating the yarns with steam may be carried out in any desired manner. For 60 example, the yarn wound on bobbins may be subjected to the action of steam at the desired temperature and pressure in a closed chamber. Thus the bobbins may be placed in a suitable air-tight chamber and after evacuating the air therefrom 65 steam may be admitted. In this way very

thorough impregnation of the yarn by the steam, which may be used for instance at a pressure of say 3 to 4 lbs. per square inch, is carried out very quickly. Instead however of evacuating the air from the chamber, means may be provided for circulating steam through the same in such a way as to displace the air from the yarn on the bobbins and ensure that every part of the yarn is effectively subjected to the action of steam. The first mentioned method is in general to be preferred however as by this process the operation is very quickly effected and there is little risk of different parts of the yarn on the bobbins or other packages being subjected to different periods of steaming or steaming under different conditions. 10 15

In order to facilitate the steam treatment, the yarn may be wound on perforated bobbins or the like in order to aid the passage of the steam into the mass of yarn. Further, in the case of such bobbins the latter may be mounted on suitable 20 perforated tubes or the like in order that steam may be blown or sucked through the yarn packages under suitable pressure from the interior to the outside or vice versa. The yarn packages may of course be wound in such a manner as to 25 facilitate the passage of steam, e. g. they may be cross wound.

Instead of effecting the steaming or like treatment of the yarn while wound on to bobbins or in other package form, the yarns may be treated 30 while travelling, for example in the course of a winding operation and particularly in the course of one of the twisting operations utilized to apply the requisite twist to the yarn. Thus, for instance, a yarn may be twisted in a machine 35 of the type in which twist is applied as the yarn is drawn off from a bobbin or like package, the yarn being subjected to the action of a jet of steam as it passes to the winding device. Conveniently the yarn may be passed through a suitable 40 chamber which may for instance take the form of a tube supplied with steam of the desired temperature. If desired the steam may be applied to the yarn at the point at which the twist is actually applied. For this purpose, in the case 45 of using a twisting machine of the aforementioned character the thread guide immediately above the bobbin from which the yarn is drawn off may be mounted at the point of entry of the yarn into the tube or like chamber in which the 50 steam is applied, or the thread guide may actually be within the said tube or like chamber. Preferably the steam is applied only in the minimum quantity necessary to secure the desired effect on the yarn in order that escape of steam and the 55 consequent likelihood of troubles arising from the rusting of machinery and the like may be avoided as far as possible.

If desired hygroscopic or deliquescent substances or wetting agents i. e. agents facilitating 60 the wetting of solids by water, may be applied to or incorporated in the yarns prior to a twisting operation or a steaming or like treatment with water vapor. As examples of such wetting agents may be mentioned soaps of organic or inorganic 65 bases with higher fatty acids, for example alkali metal, ammonium or ethanolamine soaps, sulphonated oils, sulphonic acids of alkyl naphthalenes for example butyl naphthalene sulphonate acid, and sulphonate acids or sulphuric esters of 70 higher aliphatic alcohols or of mineral oils, tar oils and the like. Mention may also be made of wetting agents of a basic character, for example the higher poly-amines of the aliphatic series and basic derivatives of the higher fatty acids. for 75

instance oleyl derivatives of aliphatic diamines or other higher fatty acid derivatives of this character.

Such hygroscopic or deliquescent substances or wetting agents may be applied to the yarns, or if desired may be incorporated in spinning solutions from which the yarns are prepared. For example, cellulose acetate solutions containing hygroscopic substances, for instance sodium or potassium acetate or calcium or magnesium chloride or nitrate may be spun into filaments and the latter formed into yarns and treated in accordance with the invention.

After the operation of steaming or the like the 15 yarn may be allowed to stand for a time. Further twist may be applied to the yarn directly or after subjecting the yarn to a drying operation in order to remove a part or the whole of any moisture content. The proportion of moisture remaining prior to the further twisting operation 20 or operations may be adjusted to that most favourable to the production of the yarn giving good crêpe fabrics. The aforementioned drying of the yarn, where desired or requisite, may be effected in any convenient manner. For example, the yarn may be passed over heated drums or through another suitable drying device after treatment but prior to rewinding, or it may be subjected to diminished pressure, e. g. on bob- 25 bins or the like.

Cellulose acetate yarns to which a high degree of twist has been applied in the manner described, may be incorporated into fabrics and the latter subjected to a scouring operation or like 30 aqueous treatment.

It appears possible that the improved results obtainable in accordance with the new process are to be attributed to the application of at least 35 part of the high twist to a yarn of more or less firm character in which the filaments are bedded firmly together, tend to retain their relative positions, and are not subject to substantial relative movement during twisting. Such a yarn, in which the filaments may be described as being 40 "set", when further twisted appears to twist substantially as a whole, the applied twist causing the 45 yarn to assume a spiral form. Further it may be that the treatment with water vapour serves to soften the material of the filaments to some extent and so remove strain therefrom and permit 50 the production of a yarn of the foregoing character. We have indeed found that the water vapour may be replaced wholly or in part by other 55 vapours especially of substances having a softening action, particularly a very mild softening action on the material of the filaments. The 60 vapours may be applied at temperatures in the neighbourhood of the boiling point of the particular substance or at lower or higher temperatures. As examples of such substances mention 65 may be made of alcohols, for example ethyl or methyl alcohol, halogenated hydrocarbons, for example ethylene dichloride or carbon tetrachloride, esters for instance ethyl acetate, or mixtures 70 of the foregoing substances with one another or with other substances. The substances should preferably not however be of such character or applied under such conditions as would cause solution or even any very material softening of 75 the substance of the filaments.

Again, we have found that instead of using water or other substance in vapour form the water or other substance may be applied in the form of a fine spray. Thus for instance instead of applying steam to the yarn, for example dur-

ing or immediately following a twisting operation, a very fine spray of water, which may be heated, may be applied to the yarn. As in the case of steam or other vapours such spray of water or other softening liquid may be applied in restricted quantity so as to avoid as far as possible any rusting of the machinery. The spray may for instance be applied in a closed chamber, for example a chamber of tubular form through which the yarn is passed. The apparatus previously referred to as suitable for use in applying steam may be employed if desired.

Whatever the character of the treatment applied, hereinafter referred to as a conditioning treatment, it should be such as will facilitate the 15 bedding together of the filaments of the partially twisted yarn, and the production of a firm yarn adapted to receive the remaining portion of the high degree of twist.

In addition to the treatment with steam or other vapour or a spray of water or other liquid, the yarn may be subjected to any other desired treatment designed to enhance the crêpe effects ultimately obtainable. For example the yarn may be wetted, in the manner described in application Ser. No. 611,922 filed on even date here-with prior or subsequent to steaming, or again where twisting is accomplished in more than two stages the yarn may be wetted between some 25 pairs of consecutive twisting stages and steamed 30 or the like in between other pairs of consecutive twisting stages.

The crêpe threads employed in accordance with the present invention may if desired be 35 sized at any suitable stage of their manufacture, for example prior to the application of any substantial degree of twist. In this connection particular mention may be made of sizing materials selected in accordance with the principles laid down in U. S. application S. No. 491,070 filed 24th 40 October, 1930. Again, the crêpe threads or the filaments contained therein may be sized with or provided with a coating of a cellulose or a cellulose derivative as described in U. S. Pat. No. 1,993,992, or with a coating of a polymerized 45 vinyl compound or other polymerized or condensed organic compound, for example a synthetic resin, as described in U. S. application S. No. 514,898, filed 10th February, 1931. Such sizes or coatings may be applied intermittently 50 to the yarns, as described in U. S. application S. No. 559,210, filed 25th August, 1931 and Pat. No. 1,966,440.

If desired lubricants may be applied to the 55 yarns which are to receive the high degree of twist, especially while the yarns have no twist or at any rate only a low degree of twist. Such lubricant, for example, olive oil or castor oil or oleic acid, assists the filaments to slide easily 60 over each other so that they may more readily take up their proper position in the yarn, particularly during the early stages of twisting, prior 65 and up to the point at which close packing is reached. Such lubricant may be permitted to remain in the yarns throughout the twisting, when it may be removed after incorporation of the yarns in fabrics, or removal of the lubricant may be effected before the final amount of twist 70 is applied.

Fabrics containing highly twisted yarns prepared in accordance with the invention may if desired be subjected to a treatment adapted to swell the material of the filaments of the said 75 yarns. Such swelling treatment may be effected

for instance in the manner described in U. S. applications S. No. 527,358 filed 2nd April, 1931 and U. S. Pat No. 1,995,296. If desired the agent employed in the aforementioned conditioning treatment of the yarn during the twisting operation may be one capable of swelling the material of the filaments in the presence of water. As an example of such an agent ethyl alcohol may be mentioned. In such cases swelling of the material may thus be effected during the aqueous treatment, which is in general applied to the fabrics containing the highly twisted crêpe threads.

As stated previously the invention is of particular value in connection with the production of crêpe fabrics with the aid of highly twisted yarns consisting of cellulose acetate filaments. Crêpe threads comprising filaments of other organic derivatives of cellulose may be employed in an analogous manner. As examples of such cellulose derivatives may be mentioned cellulose formate, propionate or butyrate or other cellulose esters of organic acids, or methyl, ethyl or benzyl cellulose or other cellulose ethers. If desired crêpe threads consisting of or comprising filaments of other materials may be employed, for example filaments of silk, cotton, or of artificial silk of the regenerated cellulose type. The crêpe threads may also be composed of filaments of two or more different kinds whether in respect of material or denier or both. Thus there may be used threads containing both filaments of cellulose esters or ethers and filaments of natural silk or regenerated cellulose artificial silk, or threads containing cellulose ester or ether filaments of two or more different deniers, or threads containing filaments of one cellulose derivative e. g. an ester in admixture with filaments of another cellulose derivative e. g. an ester of different ester content or an ether. Further the crêpe yarns may consist, wholly or in part, of "staple fibre", i. e. relatively short lengths of filaments.

The highly twisted crêpe threads may be incorporated in the fabrics in any suitable manner, for example the weft alone may be wholly or partially composed of such threads or the warp may also contain them. In the former case the finished fabrics exhibit the greater shrinkage in the direction of the weft. It is found particularly convenient however, in general, to employ threads of relatively low twist in the warp and to employ in the weft both crêpe threads having a left-hand twist and crêpe threads having a right-hand twist. Such threads may be disposed in the fabrics in any convenient manner, for example pairs of threads of left-hand twist may alternate with pairs of threads of right-hand twist. A further method of constructing the fabrics is to weave composite crêpe threads consisting of a yarn of high twist doubled with a yarn of low twist, or consisting of two yarns of high but opposite direction of twist, the yarns being prepared and the fabrics subsequently treated in accordance with the processes of the invention. In this manner crêpe fabrics may be readily produced without the necessity for the employment of a loom capable of weaving two different types of yarn such as is necessary when alternate picks of yarn of left-handed twist and yarn of right-handed twist are to be woven. In this connection reference is made to U. S. application S. No. 444,619, filed 15th April, 1930 and U. S. application S. No. 589,304, filed 27th January, 1932.

Where the fabrics comprise yarns of low twist,

the latter may be either of the same material or of a different material from that of the highly twisted crêpe threads. For example, where the crêpe threads are composed of cellulose acetate filaments, the said yarns of low twist may be composed of cotton or of a regenerated cellulose type of artificial silk.

In the case of fabrics containing low twist yarns as well as the highly twisted crêpe threads, such yarns, particularly when forming the warp of the material, will usually be sized. In this event it has been found beneficial to employ sizes which are easily removed or at least easily softened by the scouring or like treatment subsequently applied to the fabrics after weaving. Indeed, if desired the said treatments may be modified, for example in respect of temperature or other conditions, or a special treatment may be applied, for the purpose of softening or removing the size on the yarn of low twist. Preferably the size on the said low twist yarn should be more easily softened or removed than any size which may have been applied to the highly twisted crêpe threads in the fabrics. Again, when utilizing yarns of low twist in conjunction with the crêpe threads of high twist, the said low twist yarns may be of such character or be so treated as to be less readily wetted than the crêpe threads. For instance they may be oiled with an animal, vegetable, or mineral oil prior to incorporation in the fabrics.

The invention is illustrated but not limited by the following example:—

#### Example

Cellulose acetate yarn of 100 denier and containing 26 filaments possessing say 2-5 turns per inch of twist is twisted up to 26 turns per inch and simultaneously wound on to perforated metal bobbins. The bobbins of yarn are then steamed for 5 minutes at 2 to 3 lbs. pressure and thereafter the yarn is twisted up to 70 turns per inch with the aid of the device described in U. S. Patent No. 1,784,581. Yarn of right-hand as well as yarn of left-hand twist is prepared. The prepared yarn is then woven into a warp of cellulose acetate yarn of low twist, two picks of left hand twist yarn alternating with two picks of right hand twist, the resulting fabric being then treated first in water at 30° C. for 15 to 30 minutes and thereafter in a three grams per litre soap solution for 1-1½ hours, the temperature being raised from 30 to 80° C. The fabric is finally washed off, hydroextracted and dried without tension.

Fabrics may similarly be produced from cellulose acetate yarns of other deniers and containing different numbers of filaments, the degree of twist applied in the two stages being adjusted according to the particular yarn.

What we claim and desire to secure by Letters Patent is:—

1. Process for the production of threads having a crêpe twist from textile threads which comprises applying a part only of the crêpe twist, said part amounting to at least 10 turns per inch, subjecting the thread to the action of a hot vapor and thereafter applying the remainder of the requisite crêpe twist.

2. Process for the production of threads having a crêpe twist from textile threads which comprises applying a part only of the crêpe twist, said part amounting to at least 10 turns per inch, subjecting the thread to the action of steam and thereafter applying the remainder of the requisite crêpe twist.

3. Process for the production of threads having a crêpe twist from textile threads containing filaments of organic derivatives of cellulose which comprises applying a part only of the crêpe twist, 5 said part amounting to at least 10 turns per inch, subjecting the thread to the action of steam and thereafter applying the remainder of the requisite crêpe twist.

4. Process for the production of threads having a crêpe twist from textile threads containing filaments of organic derivatives of cellulose which comprises applying to the threads a part only of the crêpe twist, said part amounting to at least 10 turns per inch, subjecting the threads to the 10 action of steam and thereafter applying the remainder of the requisite crêpe twist.

5. Process for the production of threads having a crêpe twist from textile threads containing filaments of organic derivatives of cellulose which 20 comprises applying a part only of the crêpe twist, said part being sufficient to effect the close packing of the filaments of the thread, subjecting the threads to the action of steam and thereafter applying the remainder of the requisite crêpe twist.

25 6. Process for the production of threads having a crêpe twist from textile threads containing filaments of organic derivatives of cellulose which comprises applying to the threads a part only of the crêpe twist, said part amounting to at least 10 turns per inch, subjecting the threads to the action of steam and thereafter applying the remainder of the requisite crêpe twist in a single stage.

30 7. Process for the production of threads having a crêpe twist from textile threads containing filaments of cellulose acetate which comprises applying a part only of the crêpe twist, said part amounting to at least 10 turns per inch, subjecting the threads to the action of a hot vapor and 40 thereafter applying the remainder of the requisite crêpe twist.

35 8. Process for the production of threads having a crêpe twist from textile threads containing filaments of cellulose acetate which comprises applying to the threads a part only of the crêpe twist, said part amounting to at least 10 turns per inch, subjecting the threads to the action of steam and thereafter applying the remainder of the requisite high twist.

45 50 9. Process for the production of threads having a crêpe twist from textile threads containing filaments of cellulose acetate which comprises applying a part only of the crêpe twist, said part being sufficient to effect the close packing of the

filaments of the thread, subjecting the threads to the action of steam and thereafter applying the remainder of the requisite crêpe twist.

10. Process for the production of threads having a crêpe twist from textile threads containing filaments of cellulose acetate which comprises applying to the threads a part only of the crêpe twist, said part amounting to at least 10 turns per inch, subjecting the threads to the action of steam and thereafter applying the remainder of the requisite crêpe twist in a single stage.

15 11. Process for the production of threads having a crêpe twist from textile threads containing filaments of cellulose acetate, which comprises applying to the threads a part only of the crêpe twist, said part amounting to at least 10 turns per inch, steaming the threads at 0-5 lbs. pressure above that of the atmosphere and thereafter applying the remainder of the requisite crêpe twist.

20 12. Process for the production of threads having a crêpe twist from cellulose acetate threads of from 70-170 denier and containing 25-70 filaments which comprises twisting the threads to between 10 and 30 turns per inch, subjecting the threads to the action of steam and thereafter applying the remainder of the requisite crêpe twist.

25 13. Process for the production of threads having a crêpe twist from textile threads containing filaments of organic derivatives of cellulose which comprises applying a part only of the crêpe twist to the thread, said part amounting to at least 10 turns per inch, steaming the thread, forming the thread into a package, and then applying the remainder of the crêpe twist by rotating said package and drawing the thread off over the end of the rotating package while preventing twist from running back to the package.

30 35 40 45 50 14. Process for the production of threads having a crêpe twist from textile threads containing filaments of cellulose acetate which comprises applying a part only of the crêpe twist to the thread, said part amounting to at least 10 turns per inch, steaming the thread, forming the thread into a package, and then applying the remainder of the crêpe twist by rotating said package and drawing the thread off over the end of the rotating package while preventing twist from running back to the package.

WILLIAM ALEXANDER DICKIE.  
ROBERT WIGHTON MONCRIEFF.